

Nov. 25, 1930.

**U. A. GARRED**

1,782,418

## RECOVERING METALS

Filed April 8, 1927

4 Sheets-Sheet 1



*INVENTOR*

Ulysses A. GARRED.

BY  
D. Anthony Usina, ATTORNEY

Nov. 25, 1930.

U. A. GARRETT

1,782,418

## RECOVERING METALS

Filed April 8, 1927

4 Sheets-Sheet 2



*INVENTOR*

50 BY ULYSSES A. GARRETT.  
S. Anthony Maria, ATTORNEY

Nov. 25, 1930.

U. A. GARRED

1,782,418

RECOVERING METALS

Filed April 8, 1927

4 Sheets-Sheet 3



INVENTOR

ULYSSES A. GARRED.

BY  
*R. Anthony Maina, ATTORNEY*

Nov. 25, 1930.

U. A. GARRED

1,782,418

RECOVERING METALS

Filed April 8, 1927

4 Sheets-Sheet 4

*Fig. 6.*



*Fig. 7.*



INVENTOR

BY ULYSSES A. GARRED.

*D. Anthony Mine, ATTORNEY*

## UNITED STATES PATENT OFFICE

ULYSSES A. GARRED, OF JACKSON HEIGHTS, NEW YORK, ASSIGNOR TO ANACONDA COPPER MINING COMPANY, A CORPORATION OF MONTANA

## RECOVERING METALS

Application filed April 8, 1927. Serial No. 181,979.

In a previous application No. 97,840, filed March 27, 1926, I have described a process of recovering metals from slags and other materials by forcing through the material a mixture of finely divided fuel and air.

The present application is a continuation in part thereof with certain additional features.

The accompanying drawings illustrate an embodiment of the invention.

Fig. 1 is a flow sheet of the various apparatus and stages of the process;

Fig. 2 is a longitudinal vertical section of the vessel in which the blowing takes place; Fig. 3 is a partial plan and partial section of the same on the line 3—3 of Fig. 2;

Fig. 4 is a front elevation of the same;

Fig. 5 is a side elevation of a portion of the same;

Fig. 6 is a vertical sectional view through a tuyère and connections;

Fig. 7 is a similar view illustrating a modification.

In many smelting operations it is common to lose considerable values in the slag. For example, in the operation of lead smelters slags containing considerable amounts of zinc are commonly thrown away; and corresponding losses of tin, lead and other metals are common in smelting copper and like operations.

The object of the present invention is to provide means whereby the metal may be recovered from such slags and other material.

By the present method, hot slag from the blast furnace is charged into the vessel which I call a "converter." Or, less advantageously, cold broken slag may be placed in the converter and melted.

Pulverized coal or oil or gas or similar finely divided fuel is forced, together with a quantity of air, into the converter underneath the molten slag. The fuel ignites and with the air rises through the slag. The result is a thorough mixture of the slag with the burning fuel and air. The burning fuel produces enough heat to keep the slag molten in spite of the cooling effect of the air, and

at the same time acts as an agent to assist in separating out the metals from the slag.

In the case of zinc, for example, the burning coal volatilizes the zinc (first converting it to free metallic zinc) which thereafter combines with the air and is carried off in the fumes so as to be easily recoverable in a bag house, collecting tower or similar apparatus, as zinc oxide. Other metals may be similarly obtained by volatilization.

The lead and zinc or other metals must first be reduced from the oxide before they can be eliminated from the slag, and this I effect by using an amount of coal dust greater than that which can be burned by the amount of air supplied. The excess of carbon reduces the zinc oxide to metallic zinc, which vaporizes at the temperature in the converter and is thereafter reoxidized. Also the excess of carbon remaining in the gas which passes off is oxidized.

The quantity of fuel and air to be employed depends on the nature of the material, but in all instances it is desirable to force in enough air to contact thoroughly with the slag and enough fuel to maintain the slag in unchilled molten condition and to contribute the chemical or reducing action promoting separation of the metal. This is especially important in recovering zinc, to the recovery of which the invention is particularly applicable.

An example of the process applied to the recovery of lead and zinc oxide fumes from lead blast furnace slag is illustrated in Fig. 1. Three slag furnaces or converters 1 are illustrated. The material for treatment comes in at one side on the line 2 and the waste slag is carried out on what we call the front side as indicated by the line 3. A flue 4 for the gases and fume extends over the three slag furnaces. In this flue there is further oxidation or combustion of the metals and of the carbon or carbon monoxide. The very hot gas and fume is then carried by a line 5 to a boiler or set of boilers 6 in which steam is generated and the gas and fume are at the same time considerably cooled. The cooled gas and fume pass out by a line 7 which indicates a flue of steel for effecting the complete cooling required before the metal oxides can be re-

covered. This cooling flue leads by two branches to compartments 8 and 9 of the bag house with dampers 10 and 11 by which the fume can be led to first one and then the other compartment. The oxides recovered 5 pass from the bag house by the line 12; the gas passes by the line 13 to the stack 14.

The bag house illustrates an improvement 10 which is the invention of Frederick Laist and covered in a separate application pending in his name; by which the fumes are switched 15 from one point to another at different stages of the blowing of a charge, eliminating impurities and collecting products which are more or less rich in the percentage content of lead.

The passing of the fume through the boiler 6 serves the double purpose of cooling it to approximately the degree required and of utilizing 20 the heat of vaporization and the heat of combustion of the metals and fuel within the flue.

The boiler may be used for various purposes. I have illustrated it as supplying 25 steam through a line 15 to an air compressor and water pumping plant 16. The compressed air passes through the line 17 to the slag furnaces. Water passes from the pumps through the line 18 to the slag furnaces for 30 water cooling various parts as described hereinafter.

The hot water overflowing from the cooling jackets passes out by the line 19 and the feed water line 20 to the boiler and by the line 35 21 to the cooling tower 22 where it is cooled sufficiently to be passed through the line 23 to the pumping plant.

Assuming pulverized coal to be used as fuel, the pulverizing plant 24 is used to supply 40 coal along the line 25 to the slag furnaces and along the line 26 to the blast furnaces.

The invention may be applied to various materials containing metal oxides such, for example, as cold slag taken from a dump or 45 bin as previously explained, or it may be applied to slag coming directly molten from blast furnaces.

In Fig. 1, three different materials are shown. The line 27 indicates the introduction 50 of any such material containing zinc, assuming this to be the metal we are seeking to recover. The line 28 indicates slag coming from the set of lead blast furnaces 29. The lead slag from the dump 30 may be carried 55 directly to the slag furnaces. But there are certain advantages in carrying it to the blast furnaces as indicated by way of the line 31.

In the blast furnaces it is mixed with the usual charge of lead ore. A twofold advantage 60 results from this step, and is beneficial to the operation of the blast furnaces, first in increasing the total tonnage treated by them so as to secure an increased output of lead, and the slag produced is lower in lead content than that which would be produced 65

from the ordinary charge. It is assumed that the slag contains enough zinc to make it economically worth while. By passing the slag from the dump through the blast furnaces in this way there is probably an economy in the 70 actual cost of melting compared with the separate melting of the dump slag alone.

The preferred form of converter is shown 75 in Figs. 2 to 6. The hearth is made of a layer of silica 32 with a superposed layer of magnesite brick 33. The sides 34, ends 35 and 36 and roof 37 and uptake 38 are made of hollow steel sections through which water is circulated to keep them cool and to resist the corrosive action of the molten charge. The 80 uptake from each converter is covered by an arch 39 of brick-work which is extended to form part of the common flue 40 (Fig. 4). The uptake 38 extends across the full width 85 of the converter about half way between the front and the back.

At the rear of the roof there is an opening 90 40 above which is a hopper 41 through which the molten charge is introduced from ladles, after which the opening is closed by a damper 42. At the front side of the uptake 38 there are openings 43 (Fig. 4) to admit air for oxidizing the escaping gas and fuels. In the front wall there are tapping ports 44 made in water cooled cast blocks 45.

The barren slag after a blow will be tapped and run off into chutes 46 for any convenient disposal. Also in the front wall there is a peep-hole ordinarily covered by a slide 47 of fire-brick.

The introduction of air and fuel is at numerous points along the lower parts of the two side walls 34. For this purpose two degrees of air pressure are preferred and the tuyères are constructed accordingly. There are high pressure air lines 48 and 49 on opposite sides and low pressure air lines 50 and 51, provided with the usual stop cocks. The high pressure line carries the powdered coal. The low pressure line carries such additional air as is required.

Each tuyère 52 passes through the two spaced plates 53 which constitute the side wall (Fig. 6). Each tuyère at its outer end is continued in a fitting 54 having lateral connections to a branch 55 from the high pressure pipe and to a branch 56 from the low pressure pipe and also to a branch 57 constituting a slag pocket normally protected by a fuse 58 which will burn out and permit the escape of any molten slag which backs up into the tuyère. At its outer end the fitting 54 has a punch rod opening closed by a plate 59 which is pivoted to permit swinging inward but not outward so that the pressure 115 of air will hold it closed.

Fig. 7 illustrates in vertical section a fragment of an ordinary tilting converter with a rounded bottom. The shell 60 is stiffened by vertical braces 61 and lined with magne- 120

site brick or similar refractory material 62 through which the tuyères 63 extend, terminating at its inner face. At the outside there is a main 64 carrying air at low pressure and communicating by pipe 65 with a fitting 66 on the outer end of the tuyère which has a check valve 67 closing a hole 68 through which a poker or clearing bar can be introduced in case the tuyère is choked at its inner end. 5 This is similar to the opening and valve 59 of Fig. 6. The pipe 69 carries the high pressure air and powdered coal which pass therefrom through a branch pipe 70 to the tuyère. It has been previously proposed to blow 10 coal dust through a bath of slag with an air current, but without pointing out the proportions and without sufficient information in detail to enable one to carry out the process successfully. I have ascertained by considerable experimentation on a practical scale that 15 for practical success it is necessary to carry out the process under the conditions herein described and hereinafter claimed.

Various other modifications of the process 20 and apparatus may be made by those skilled in the art without departing from the invention as defined in the following claims.

What I claim is:

1. In the recovering of volatile metals 25 from slag and the like, the method which consists in forcing through the molten slag finely divided fuel and air, introducing the fuel with air under high pressure and introducing air separately under low pressure 30 and collecting the resulting fume.

2. In the recovering of volatile metals 35 from blast furnace slags, the method which consists in adding cold slag to the charge of the blast furnace, carrying the molten slag from the blast furnace to a slag furnace, 40 forcing through such molten slag finely divided fuel and air and collecting the fume.

3. In the recovering of volatile metals 45 from blast furnace slags, the method which consists in adding cold slag to the charge of the blast furnace, carrying the molten slag from the blast furnace to a slag furnace, adding to the charge in the slag furnace cold material containing the metal to be recovered 50 and forcing through the charge in the slag furnace finely divided fuel and air sufficient to maintain the charge molten and collecting the fume.

In witness whereof, I have hereunto 55 signed my name.

ULYSSES A. GARRED.